

March 8, 1938.

B. H. THURMAN

2,110,780

PROCESS OF TREATING DRYING OILS TO BODY SAME FOR VARNISH AND OTHER USES

Original Filed July 19, 1933



## INVENTOR

Benjamin F. Thierman

BY

Gifford, Seale & Burgess ATTORNEYS

## UNITED STATES PATENT OFFICE

2,110,780

PROCESS OF TREATING DRYING OILS TO  
BODY SAME FOR VARNISH AND OTHER  
USESBenjamin H. Thurman, Bronxville, N. Y., assign-  
or, by mesne assignments, to Refining, Inc.,  
Reno, Nev., a corporation of NevadaApplication July 19, 1933, Serial No. 681,048  
Renewed August 30, 1937

6 Claims. (Cl. 87—12)

This invention relates to a process of treating fish and vegetable oils for the purpose of bodying them or preparing them to be used in the paint and varnish industry and for making 5 enamel, linoleum, etc.

Heretofore, oils have been heated in open kettles over a fire for the purpose of bodying them. This requires a high degree of skill on the part of the operator as the oil is not sufficiently 10 bodied if the heating is not carried far enough and the oil becomes darkened if it is exposed to the air too long at the elevated temperature.

It requires a long time to impart sufficient body to the oil by the former heat treatment. For 15 example, it requires several hours to increase the specific gravity of linseed oil from about 0.936 to 0.962 and the viscosity from about 2.2 to 47 by the Ford cup test viscometer, in this old way. During this long time of treatment the oil often 20 becomes discolored to an objectionable extent.

Also, gums or resins that are added to the vegetable oils in making varnish, etc. usually have to be heated to 550° F. to 600° F. to remove volatile materials that will not mix satisfactorily 25 with the vegetable oils in varnish making. They sometimes amount to 10% to 20% of the weight of the gums or resins. If these volatile products are not removed they cause the varnish to become cloudy.

30 By the present invention oils, gums and resins that are to be used in varnish and other industries are heat-treated in such a manner that the proper amount of body is imparted to them or the desired amount of volatile materials is re- 35 moved very rapidly without imparting the other usual objectionable properties.

In carrying out this invention the oil or gum to be treated is passed rapidly through a heated coil under pressure where it undergoes consider- 40 able stirring or agitation while it is being heated and it is then permitted to expand into a receiver at a lower pressure whereupon the volatile constituents flash into vapor.

The invention will be explained in connection 45 with the accompanying drawing which shows an arrangement of apparatus for practicing the process. In the drawing Fig. 1 is a somewhat diagrammatic arrangement of apparatus for carrying out the invention and Fig. 2 is a longitudinal section on an enlarged scale partly broken away showing a modification of one of the details.

In the drawing reference character 1 indicates a tank or receptacle for the material. This tank is provided with a stirrer and may be heated 50 in any convenient way, if desired.

A pipe 3 having a valve 4 leads from the lower portion of the tank 1 to a pump 5 from which a pipe 6 leads to a coil 7 in the heater 8. The lower end of the coil 7 opens into an automatic heat regulator 9.

The heat regulator 9 comprises an elongated hollow member 10 extending across the lower end of the heater 8, with an inner tube 11 anchored at its closed end 12 in the hollow member 10. The other end 13 of the tube 11 is open and the walls are slitted and spread out so that the ends of the slits contact with the inside surface of the hollow member 10 leaving openings for material to pass from the annular space 14 between the tube 11 and member 10 into the tube 11. 5

One end of the heat regulator 9 is held in ad- 10 justed position by the threaded support 15 pass- 15 ing through a threaded opening 16 in a wall of the heater 8. An enlarged head or hand wheel 17 is provided on the outer end of the support 15 20 for turning it. The inner end of the support 15 terminates in an enlargement 18 revoluble in a recess 19 provided therefor at the closed end of the member 10, so that the heater 9 can be moved 25 longitudinally into different positions by means of the support 15.

The end of the member 10 opposite the support 15 carries a stem or extension 20 which extends 30 through an opening 21 in the wall of the heater 8 and supports that end of the heat regulator 9. 30 A valve 22 is fixed on the outer end of the stem 21 in a housing 23 that is attached to the wall of the heater 8 and carries a valve seat 24. A pipe 25, having a valve 26, for fluid fuel, such as gas, is connected to the housing 23 on the side of the 35 valve seat 24 opposite the valve 22. An outlet pipe 27 leads from the other side of the valve seat 24 to the burner 28.

An outlet pipe 30 having a valve 31 leads to a junction 32 from which a pipe 33 having a valve 34 leads to a nozzle 35 in an expansion cham- 40 ber 36. A cylindrical extension 37 having its lower end open surrounds the nozzle 35. The expansion chamber is provided with a stirrer 38 and a valved outlet pipe 39.

An outlet pipe 40 for gas or uncondensed va- 45 pores leads from the upper portion of the cham- 45 ber 36 to a condenser 41 cooled by the cooling coil 42. A valved outlet pipe 43 for condensates 50 is connected to the lower portion of the con- 50 denser 41 and a pipe 44 for uncondensed gases leads from this condenser to a liquid seal tank 45.

A pipe 46 having a valve 47 leads from the junction 32 to the tank 1. A pipe 48 having a valve 49 leads from the pipe 3 to a coil 50 in the 55

chamber 36. A pipe 51 having a valve 52 leads from the coil 50 to the pipe 3 on the other side of the valve 4 from the pipe 48.

In the modification indicated in Fig. 2, the 5 pipe 30 leads to a jacket 55 surrounding the pipe 3 so that the material flowing through the pipe 3 becomes heated by the hot material passing through the pipe 30.

In carrying out the invention the oil or other 10 material to be bodied or heat-treated is introduced into the tank 1 through the opening 1' and may be heated to some extent in this tank, if desired. The oil passes from the tank 1 through pipe 3 to the pressure pump 5 and thence 15 to the heating coil 7. The pressure in the coil 7 is maintained at the desired point to prevent or limit volatilization or constituents by regulating the valve 31 or by use of a properly restricted nozzle 35 in the tank 36.

20 The oil, or other products, is heated to the desired extent in the coil 7 by the products of combustion from the burner 28, the waste products of combustion escaping through the outlet 8'. The material rapidly changes direction of travel 25 in the coil 7, thus causing the same to be stirred or agitated so that it is uniformly heated. The heated material passes from the coil 7 into the annular space 14 in the heat regulator 9 and thence through the passages 13 into the tube 11 30 from where it passes through the pipe 30 to the nozzle 35. The release of pressure at the nozzle 35 causes volatile constituents to flash into vapors leaving the unvaporized portions in the tank 36, from which they may be withdrawn through the 35 outlet 39. The vapors pass through the pipe 40 to the condenser 42, from which the condensates may be withdrawn through the outlet pipe 43. Uncondensed vapors or gases pass out through the pipe 44 and liquid seal 45.

40 The heat regulator 9 is automatic as increased temperature causes the member 10 to expand and move the valve 22 nearer its seat 24, thus shutting off a portion of the fuel gas entering the burner 28 from the pipe 25. A decrease in 45 the temperature of the heater 9 causes it to contract and move the valve farther from its seat 24, thus admitting more gas to the burner 28. By adjusting the support 15, the temperature may be regulated at any desired point.

50 The valve 4 may be closed and the valves 49 and 52 opened so that the material on the way to the pump 5 from the tank 1 passes through the coil 50 and is thereby heated by the hot material in the tank 36. The stirrer 38 facilitates transfer 55 of heat from the hot material in the tank 36 to the cold material in the coil 50.

Instead of providing the coil 50 in the tank 35, the jacket 55 (Fig. 2) may be provided so that heat is transferred from the material as it passes 60 from the heat exchanger 9 to the nozzle 35.

In case it is desired to pass the material through the coil 7 more than one time before it is passed to the tank 36, this may be done by closing the valve 34 and opening the valve 47, the valve 31 65 being adjusted to regulate the pressure that is desired in the coil 7.

The specific gravity and viscosity of linseed oil, for example, increases gradually, when it is heated, but China-wood oil becomes solidified 70 when it is heated for a few minutes, say 11 to 15 minutes, at about 580° to 600° F. However, China-wood oil can be heated in the apparatus described above from room temperature, 70° F. to about 625° F. in a few seconds and then cooled 75 suddenly without danger of its becoming solidi-

fied. When so treated it loses its property of becoming solidified by heating it to the temperature and for the time required for bodying it. This treatment avoids the necessity of adding other oils, such as linseed or soya bean oil, or 5 resins to it to enable it to be cooked or boiled without solidifying. Also, by heat-treating China-wood oil, as described, and bodying it by boiling, it does not become crinkled or frosted when it dries so that it is suitable for making varnish 10 or lacquer.

It is commonly believed that bodying oils results not only because of removal of volatile constituents but also because polymerization takes place during the heating. Even a very short time 15 of heating, as described herein, appears to produce both of these results. Polymerization increases the water-proofing qualities of the oil and permits the use of cheaper gums or resins than kauri or pontiac in making varnishes with the 20

25 By the present invention the oil is heated and bodied very effectively and efficiently in an economical manner. It requires only about six to ten minutes to increase the temperature from room temperature to the desired temperature which is about 580° F. for most oils that are used in making varnishes. However, on account of the short time that the material is kept in the coil, the temperature of the oil may be as high as 30 650° F. without great danger of injury to the oil. The oil has high velocity and turbulent flow through the coil so that rapid heat transfer to the oil takes place and local overheating is prevented.

35 Driers such as those ordinarily used in oils may be added in the tank 1 and stirred into the oil and passed with it through the coil 7. Pigments may be added in a similar way. The driers or pigments become thoroughly mixed with the oil 40 in passing through the coil 7 even if they are not so mixed before the oil enters this coil. Air is excluded from the oil while it is being heated, whether driers are present or not, and the tendency of the oil to become yellow when used to 45 make paints varnishes, etc., is decreased. Air is also excluded from the oil while it is still hot in the tank 36.

50 When it is desired to remove volatile products from gums or resins in accordance with this invention, this can be done by powdering or comminuting the resins or gums and mixing them with sufficient oil in the tank 1 for the mixture to flow. The volatile constituents pass off when the hot mixture emerges from the nozzle 35. The 55 liquid residue may be passed through the coil 7 repeatedly, if necessary, until the desired amount of volatile matter has been removed, and the right proportion of vegetable oil necessary for making varnishes can then be added in the tank 1 and 60 the mixture passed through the coil 7 and heated adequately in a few minutes to impart the desired viscosity and specific gravity. The prior method of heating in kettles required many hours, often overheated or burned the oils and gums and contact with air at the elevated temperatures often 65 caused discoloration.

70 In using this invention, oil, containing a drier, which required boiling for four hours in a varnish kettle to increase its specific gravity from 0.9316 70 to 0.9512 and then required eleven hours to become dry, required only six minutes heating by this process to produce the same increase in specific gravity and it dried in six hours. The coil used was made of a steel pipe one-half inch in- 75

side diameter and 320 ft. long. The temperature to which the oil was increased was approximately 580° F.

In another run a mixture of linseed and China-  
5 wood oil that would not dry in 24 hours and had a sp. gr. of .9465 was passed through the coil at such a rate that it was heated only six minutes without appreciable change in sp. gr. but the oil then dried in 19 hours. A sample of the same  
10 mixture passed through the coil twice under the same conditions had its specific gravity increased less than one-tenth of one per cent, but the drying time was reduced to 6 hours. It is very desirable in the paint and varnish industry to have  
15 oils that ill dry rapidly and still not have greatly increased viscosity and specific gravity. Heretofore, fast drying oils have necessarily been of high viscosity and high specific gravity.

By the present process, fish oils can be successfully treated so that they are bodied to the extent that make them suitable for use in the paint and varnish industries and at the same time the volatile constituents which impart an objectionable odor are removed. By heating such  
20 oils to temperatures of 580° F. to 600° F. while excluding contact with air they become polymerized or bodied to the desired extent.

After the material has been heated in the coil  
7 and expanded in the chamber 36 it should be  
30 allowed to cool before being withdrawn through the outlet pipe 39 wherever there is danger of the material becoming injured by contact with air while it is hot.

I claim:—

35 1. The process of treating a drying oil for making varnish and other products which comprises passing the oil through an elongated curved heated zone at a temperature sufficient to body said oil and at an elevated pressure sufficient to limit volatilization of constituents while excluding air therefrom, suddenly releasing the pressure and withdrawing volatile products.

2. The process of treating a drying oil for making varnish and other products, which comprises, passing said oil under pressure and out of contact with the air through a heated zone of such dimensions that the oil is substantially uniformly heated, raising the temperature of said oil in said zone sufficient to body the oil and to

cause volatile constituents to pass into vapor when the pressure is lowered, suddenly lowering said pressure and withdrawing said volatile constituents.

3. The process of treating a drying oil for 5 making varnish and other products, which comprises, passing said oil through a heated zone at an elevated pressure and out of contact with the air, maintaining sufficient velocity of said oil in said zone to cause the oil to be substantially uniformly heated, raising the temperature of said oil in said zone sufficient to body the oil and to cause volatile constituents to pass into vapor when the pressure is released, suddenly releasing said pressure and withdrawing said volatile constituents. 10 15

4. The process of treating a drying oil for making varnish and other products, which comprises, passing said oil at an elevated pressure and out of contact with the air through a heated 20 zone of such dimensions that the oil is substantially uniformly heated, raising the temperature of said oil in said zone to approximately 580° F., suddenly releasing said pressure and withdrawing 25 volatile products therefrom. 25

5. The process of treating a mixture of varnish adjuvants and a drying oil suitable for making varnish, which comprises, passing said mixture at an elevated pressure and out of contact with the air through a heated zone of such dimensions that the mixture is substantially uniformly heated, raising the temperature of said mixture in said zone sufficient to body the oil and to cause volatile constituents thereof to pass into vapor when the pressure is released, suddenly 30 35 releasing said pressure and withdrawing said volatile constituents.

6. The process of treating a mixture of gum and a drying oil suitable for varnish making, which comprises, passing the mixture through a 40 heated zone at an elevated temperature and out of contact with the air, raising the temperature of said mixture in said zone sufficient to body the oil and to cause substantially all of the volatile constituents of said gum to pass into vapor when the pressure is suddenly released, suddenly 45 releasing said pressure and withdrawing volatile constituents.

BENJAMIN H. THURMAN.